

# UNITED STATES PATENT OFFICE.

ALOIS SCHайдHAUF, OF FRANKFORT-ON-THE-MAIN, GERMANY, ASSIGNOR TO THE ROESSLER & HASSLACHER CHEMICAL CO., OF NEW YORK, N. Y., A CORPORATION OF NEW YORK.

## PROCESS FOR BLEACHING TEXTILE FIBERS.

1,235,929.

Specification of Letters Patent.

Patented Aug. 7, 1917.

No Drawing.

Application filed October 2, 1913. Serial No. 793,039.

To all whom it may concern:

Be it known that I, ALOIS SCHайдHAUF, a subject of the Emperor of Germany, and resident of Frankfort - on - the - Main, Germany, have invented certain new and useful Improvements in Processes for Bleaching Textile Fibers, of which the following is a specification.

This invention relates to improvements in processes for bleaching textile fibers, such as cotton, by means of alkaline hydrogen peroxid solutions stabilized by anticatalyzers.

The introduction of the strongly alkaline solutions of sodium peroxid for bleaching purposes, though easily obtainable, has met with delay because of the fact that hydrogen peroxid solutions of strongly alkaline reaction very quickly give off their oxygen.

Furthermore, those skilled in the art generally have been of the opinion that textile fibers containing cellulose could not be treated with any strongly alkaline agent giving off oxygen, without reducing their valuable properties.

In the standard text-book "*The Chemistry of Cellulose*" by Schwalbe, (1911) the following is said on page 143, viz:

"Again the strongly alkaline solutions are the most detrimental ones. Here sodium peroxid stands in the front line. If dissolved in water one obtains caustic alkali besides hydrogen peroxid and the detrimental action of the former must be counteracted by the addition of acid or magnesium sulfate unless it is preferable to operate with a neutral bath as for instance for such bleaching operation, the purpose of which consists strictly in removing impurities only, without simultaneously oxidizing the cellulose-fiber."

In view of the points discussed above it has been suggested to achieve the cleaning and simultaneous bleaching of the cotton as well as of other vegetable fibers with slightly alkaline solutions of materials giving off oxygen, said solutions being produced by first neutralizing the strong alkali by a strong acid and then rendering the nearly neutral solution thus obtained alkaline by adding thereto a salt of a slight alkaline reaction. (See *Deutsche Faerberzeitung* of June 30, 1912, pg. 512-513.) This latter

process is both too cumbersome and expensive to compete with the wellknown processes using chlorin as a bleaching agent.

I have endeavored to carry out the bleaching process with strongly alkaline solutions, as obtained for instance when dissolving sodium peroxid in water, without previously neutralizing the free caustic alkali.

I have now found, that this purpose may be achieved if small quantities of a soluble magnesium salt, or small quantities of a combination of magnesia or magnesium, with silica or silicates respectively, are added to a solution of a peroxid, preferably sodium peroxid.

The addition may be made before or after preparing the solution of the sodium peroxid; one may add either ready made compounds or one may add the components of the same to effect the formation of the respective compounds in the solution of the peroxid.

With great advantage I may prevent the premature decomposition of the peroxid solution by employing the anticatalyzers in a state in which the latter are able to diffuse as much as possible within the solution, viz. by employing them in a colloidal or gelatinous form.

In preparing the peroxid solution I may also use natural water containing such anticatalyzers, and to such natural water containing an anticatalyzer in either an insufficient quantity or only one component of the same, I may add either the missing quantity of the anticatalyzer or the missing component in order to produce the anticatalytic action within the solution.

I have furthermore made the surprising discovery that the fiber is not affected in any way by treating it with solutions having a high content of free caustic alkali if the anticatalytic action, forming the subject matter of this invention, has been established in said solutions.

The following example will serve for the further elucidation of my invention. In bleaching cotton for instance I proceed as follows:

100 kilograms of cotton goods are thoroughly wetted whereby they take up 200 kilograms of water. In preparing the bleaching bath I dissolve 1.6 kilograms of

sodium peroxid in 400 liters of water. To this solution I add solutions containing each 0.15 kilograms sodium-silicate and 0.12 kilograms of magnesium chlorid, whereupon I 5 finally add 0.4 kilograms of Monopol-soap, the latter comprising a staple standard soap made by treating olive oil with caustic potash, a certain amount of Turkey red oil and carbon tetrachlorid having been added to 10 the crude soap. The bleaching bath then being ready, the wetted cotton-goods are immersed in the same.

Within the first hour the temperature is raised up to about 65-67° C. and maintained at this point for a further hour; thereupon it is raised up to about 87° C. and the bleaching is continued until the bath is exhausted.

Cottons of various origins display different behaviors in being bleached by means of oxygen, inasmuch as some become perfectly white by one single treatment, necessitating only a little more bleaching liquor, whereas others require a second treatment.

25 By the present invention I succeed in bleaching cotton perfectly white without affecting it in the least.

My new process compares very favorably with the processes using chlorin as a bleaching agent, inasmuch as chlorin is unwholesome, affects the cotton unfavorably and gives cause to losses in weight, thus rendering cotton bleached by my new process superior in every way to that bleached with 35 chlorin.

The properties of cotton bleached by the present process do not suffer in any way or manner, but, on the contrary the cotton exhibits most remarkable properties in regard to strength and elasticity.

40 In bleaching loose cotton by the present process the losses sustained in weight are very considerably lower than those by the old processes employing the old lye-boil and chlorin bleaching process. My new process is also superior to the chlorin process inasmuch as it is free from deleterious effect on the health of the workmen, and is much simpler in its operation without causing any 50 greater expense than said latter process.

It is obvious that, while I have explained my invention with reference to the bleaching of cotton and the claims are especially intended to comprehend cotton as one of the 55 fibers which may be treated by my new process, nevertheless the principles of the invention and the new process disclosed are just as applicable to other textile fibers as to cotton, as well as to other material which in the 60 modern sense of the terms "textile fiber" may be understood as such, such material being for instance straw, wood in either disintegrated form or even in the form of plates, etc. I do not restrict myself therefore, to the use of the process in connection

with the bleaching of any particular fibers further than the scope of the appended claims demands, and where in the claims I use the word "soluble" as qualifying the word "anti-catalyzer" I mean to use such 70 word in a broad sense including as well colloidal solutions.

I claim:

1. The process of bleaching textile fibers consisting in treating the fibers with a solution containing both caustic alkali and a substance carrying available oxygen, retarding the decomposition of the latter substance and simultaneously preventing decomposition of said fibers by said caustic alkali by 80 the presence of a soluble anti-catalyzer.

2. The process of bleaching textile fibers consisting in treating the fibers with a solution containing both caustic alkali and a substance carrying available oxygen and retarding the decomposition of the latter substance and simultaneously preventing decomposition of said fibers by said caustic alkali by 85 the presence of an anti-catalyzer of colloidal form.

3. The process of bleaching textile fibers consisting in treating the fibers with a solution containing both caustic alkali and available oxygen in the form of hydrogen peroxid, and retarding the decomposition of 95 the hydrogen peroxid and simultaneously preventing decomposition of said fibers by said caustic alkali by the presence of a soluble anti-catalyzer.

4. The process of bleaching textile fibers 100 consisting in treating the fibers with a solution containing both caustic alkali and available oxygen in the form of hydrogen peroxid, and retarding the decomposition of the hydrogen peroxid and simultaneously preventing decomposition of said fibers by said caustic alkali by the presence of an anti-catalyzer of colloidal form.

5. The process of bleaching textile fibers 110 consisting in treating the fibers with a solution containing both caustic alkali and a substance carrying available oxygen, retarding the decomposition of said latter substance and simultaneously preventing decomposition of said fibers by said caustic 115 alkali by the addition of a soluble magnesium compound which acts as an anti-catalyzer.

6. The process of bleaching textile fibers 120 consisting in treating the fiber with an alkaline solution containing active oxygen and a colloidal magnesium compound, the latter acting as an anticatalyzer.

7. The process of bleaching textile fibers 125 consisting in treating the fibers with a solution containing both caustic alkali and available oxygen in the form of hydrogen peroxid, and retarding the decomposition of the hydrogen peroxid and simultaneously preventing decomposition of said fibers by said 130

caustic alkali by the addition of a magnesium compound which acts as an anti-catalyzer.

8. The process of bleaching textile fibers consisting in treating the fiber with an alkaline solution containing active oxygen in the form of hydrogen peroxid and a colloidal magnesium compound acting as an anticatalyzer.

10. 9. The process of bleaching textile fibers consisting in treating the fibers with a solution containing both caustic alkali and a substance carrying available oxygen, and retarding the decomposition of said latter substance and simultaneously preventing decomposition of said fibers by said caustic alkali by the addition of a soluble combination of magnesia and silica, said combination acting as an anti-catalyzer.

20. 10. The process of bleaching textile fibers consisting in treating the fiber with an alkaline solution containing active oxygen and a colloidal combination of magnesia and silica acting as an anticatalyzer.

11. The process of bleaching textile fibers 25 consisting in treating the fibers with a solution containing both caustic alkali and available oxygen in the form of hydrogen peroxid, and retarding the decomposition of the hydrogen peroxid and simultaneously 30 preventing decomposition of said fibers by said caustic alkali by the addition of a combination of magnesia and silica, said soluble combination acting as an anti-catalyzer.

12. The process of bleaching textile fibers 35 consisting in treating the fiber with an alkaline solution containing active oxygen in the form of hydrogen peroxid and a colloidal combination of magnesia and silica acting as an anticatalyzer.

40 In testimony whereof I have signed my name to this specification in the presence of two subscribing witnesses.

ALOIS SCHAUDHAUF.

Witnesses:

JEAN GRUND,  
CARL GRUND.